

Aug. 11, 1925.

1,549,394

W. S. TYLER

RESISTANCE CONDUCTOR AND MANUFACTURING PROCESS AND MATERIAL THEREFOR

Filed Jan. 20, 1923

Fig. 1



Fig. 2



INVENTOR.

Walter S. Tyler

BY

*R. B. Whitman*  
ATTORNEY

## UNITED STATES PATENT OFFICE

WALTER S. TYLER, OF BRIDGEPORT, CONNECTICUT, ASSIGNOR, BY MESNE ASSIGNMENTS, TO COLUMBIA PHONOGRAPH COMPANY, INC., A CORPORATION OF NEW YORK.

## RESISTANCE CONDUCTOR AND MANUFACTURING PROCESS AND MATERIAL THEREFOR.

Application filed January 20, 1923. Serial No. 613,860.

*To all whom it may concern:*

Be it known that I, WALTER S. TYLER, a citizen of the United States, and a resident of the city of Bridgeport, county of Fairfield, and State of Connecticut, have invented certain new and useful Improvements in Resistance Conductors and Manufacturing Processes and Materials Therefor, of which the following, taken in connection with the accompanying drawings, is a specification.

This invention relates to resistance elements—i. e. conductors of high resistivity—capable of being calibrated to any desired resistance value, and to the method or process of producing the same.

An object of the invention is to provide a relatively high resistance unit having relatively small dimensions, and with practically no inductance or capacity, this unit being especially applicable for use in radio-receiving sets.

Another object is to provide a resistance which can be readily calibrated to a predetermined resistance value and without altering its composition; and which, moreover, is not materially affected by small or ordinary temperature changes, and yet is capable of permanent change through material variations in temperature.

A further object is to provide a resistance conductor whose resistance value may be raised by reducing its cubical contents, and yet lowered, by polishing or rubbing its surface. Also, if the resistance becomes too low by this polishing or rubbing, it may be increased by rubbing the surface with a solvent—such as alcohol—for the shellac or other binder for the conducting medium.

A further object is to provide a resistance conductor of such composition that heating it, either by an electric current, or otherwise, will increase its resistance.

Yet another object is to provide a resistance, capable of being easily molded to any desired size and shape, and which will lend itself to quantity production, at low cost.

Another object is to provide a resistance

unit structure adapted to have both a plurality of essentially predetermined resistance values, and also an easily variable resistance value.

Then, an object is to provide a resistance unit having a condenser effect.

Finally, an object is to provide a non-inductive resistance having little or no condenser effect.

With these and other objects in view, as will hereinafter more fully appear, the invention is described in the following specification, taken in connection with the accompanying drawings, in which—

Fig. 1 is a perspective view of a composite form of the invention, including all of the novel features thereof, but disclosing, of course, only the structure of the invention, the composition and process of manufacture being hereinafter brought out;

Fig. 2 is a magnified, cross-sectional view thereof, taken on the line 2—2 of Fig. 1.

In the drawings, for illustrative purposes only, the article is shown as rectangular in outline and consisting of a slab of the greater resistance material 1, having a greater conducting coating 2, this coating being formed by rubbing or polishing in manner as hereafter explained. The slab is a composite structure arranged to have the various characteristics heretofore suggested.

One part of the unit, marked B, has three binding-post terminals, 3, 4 and 5, one of which—as, for instance, 5—is movable longitudinally toward and away from the others by being mounted in a longitudinal slot formed in the unit. This is accomplished by unscrewing both the lock nut 6, Fig. 2, and the binding nut 7, on the stud screw 8, thereby releasing the conducting washers 9—9 from gripping contact with the surface of the unit, and permitting this entire binding-post assembly to be moved in its slot, and so alter the distance between the two terminals 5 and 4, or 5 and 3. Moving the terminals together reduces the resistance, and vice versa. This structure constitutes not only a novel means of calibrating the unit to any

desired value; it also provides a unit having a plurality of predetermined resistance values—as by using binding-posts 2 and 4—in combination with a predetermined range of easily variable resistance values, as by using binding-posts 4 and 5, or 3 and 5.

The other part of the unit, A, has superimposed on each of its faces an insulating or non-conducting layer 10, and superimposed 10 on these layers a conducting layer or plate 11. The binding-posts 12 and 13 are similar to posts 3, 4, and 5, except that the stud screw 14, is slightly longer to accommodate an insulated washer 15, as shown in Fig. 2; this 15 washer, in the embodiment shown, having also a hollow tubular portion 16 adapted to house the stud screw 14, and to insulate it from the unit itself. Thus there is provided a binding-post structure in which contact is made with the resistance unit on one 20 surface only. By inserting the binding-posts in part A of the unit in reverse position, as shown at 12 and 13, Fig. 1, contact is made between the top surface at 12, and 25 the bottom surface, at 13. Thus a condenser is provided in combination with the resistance unit, its effect being controlled, for instance, by the distance between the conducting plates 11—11, and the distance between 30 the terminals 12 and 13. This composite structure, with its plurality of binding-posts, provides a convenient means of getting a variety of resistance and condenser effects, simply by connecting to various pairs of 35 binding posts.

Various substances can be used for the non-conducting and the conducting elements of the compound. As the conducting element, it is preferred to use graphite. For 40 the non-conducting element, various substances or their combinations can be used, preferably a plastic composition including china clay, Congo gum, and shellac, in proportions about the same as that used in the manufacture of phonograph records—as, for 45 instance, 70%, more or less, of china clay; 5%, more or less, of Congo gum; and 25%, more or less, of shellac.

These ingredients are mixed in a finely 50 divided state, either granulated, but preferably in powdered form, the finer the ingredients the better, as it obviates any slight arcs which might form between the grains of granulated material.

To this non-conducting composition is added graphite or other conducting material in a proportion such that the approximate final resistance value of the unit will be approximately as desired. All of the ingredients, having been brought to a very fine state, are thoroughly mixed, preferably in the presence of heat and pressure, so that all the particles of the conducting material are divided or separated by particles of non-conducting material. The more inti-

mate the mixture, the better the result. The heat, when used, serves to melt the gums in the non-conducting composition; and to aid in more thoroughly mixing the various ingredients.

After the material is thus mixed, it is heated on a steam table, and formed into suitable blocks, or other units, under a set of molding dies. It is then removed and allowed to harden. The terminals may be 70 embedded within the composition at the time of pressing, or inserted afterwards.

Applicant has discovered that, in addition to the known ways of calibrating each unit to any desired resistance—such, for instance, as altering its length between terminals, or the resistance value of the material itself—the same result may be secured by removing the exterior surface of the resistance member by abrasion in such manner that no polishing effect takes place. Also, and in place of this, by the use of a solvent, such as alcohol, for dissolving away the conducting graphite coating. By thus removing the coating or skin of the member, the conductivity of the body, as a whole, is largely reduced, or, which is the same thing, the resistance increased.

Another means of calibrating the resistance unit for an increase in resistance, is to allow current to pass through it sufficiently strong to effect a heating action or to otherwise heat the unit. The shellac in the composition will be melted and caused to flow more completely around the different particles of graphite, and so effect this increased resistance.

Another means to alter the resistance value, is to actually remove sufficient of the material between terminals to appreciably alter the cross-sectional area of the unit; this also results in increasing the resistance. In the event the unit has thus had its resistance increased beyond the desired amount, a reverse calibration effect can be produced by polishing, so as to bring the graphite particles on the surface into more intimate contact.

Obviously, various kinds of ingredients, suitable for the purpose stated, will suggest themselves to those skilled in the art. Likewise, the proportions of these ingredients can be varied within quite wide limits, depending upon the characteristics of the specific ingredients used, and the distance between terminals of the resistance, and the amount of resistance desired.

Therefore, it is understood that the scope of the invention is not to be considered as limited to the particular materials, structure, and method described, but instead, solely by that covered in the appended claims.

Having thus described the nature of this invention and a preferred form and method for same, what is claimed and for which

Letters Patent of the United States is desired, is—

- 5 1. The method of manufacturing resistances, which consist in mixing a clay, a gum and a shellac with graphite, to form a thermoplastic material, in molding the composition to the desired form under the application of heat and pressure and in allowing it to cool and harden.
- 10 2. A resistance member containing a clay, a gum, shellac and graphite.
3. A resistance member consisting of a clay, a gum, a shellac, and a suitable conducting material intermixed therewith.
- 15 4. A variable resistance including a body portion of predetermined resistance, a pair of binding posts secured to said body, sheets

of insulation material spaced from the binding posts and contacting with the body, sheets of conductor material disposed on the 20 insulation, and a second pair of bolts passing through the laminated portion of the unit, and each contacting with one of the sheets of the conductor material.

5. A resistance unit containing china 25 clay, Congo gum and shellac, mixed in approximately the following proportions, china clay 70%, Congo gum 5% and shellac 25%, together with graphite.

Signed at Bridgeport, in the county of 30 Fairfield and State of Connecticut, this 18th day of January, A. D. 1923.

WALTER S. TYLER.